

## UNITED STATES PATENT OFFICE

1,942,779

## ALLOY STEEL

Hermann Josef Schiffler, Dusseldorf, Germany

No Drawing. Application December 3, 1928,  
Serial No. 323,572, and in Germany January 19,  
1928

2 Claims. (Cl. 75—1)

Alloys of iron and aluminum in themselves are known. Their use is however very limited, as although they have good properties, these are accompanied by a greater number of unfavorable ones, depending upon the amount of the content in aluminum.

4% aluminum steel has been worked up into dynamo and transformer plates in order to utilize that property of aluminum which has a similar effect to silicon on the magnetic losses of soft iron. The use of this has however been given up as the aluminum plates in other respects had not properties of the same value as the silicon sheets and were moreover more expensive.

15 German Patent No. 431,314, class 18b describes alloys which it is claimed possess the special advantages of a high electrical resistance and great resistance to heat. They contain from 8 to 16% of aluminum, 6 to 18% of chromium or 6 to 20 8% of manganese. These alloys belong to the class of high heat resisting alloys, which in general show a high percentage content of chromium and nickel, with or without other constituents, as for example, manganese, cobalt and in a few cases also aluminum between 8 and 60%.

Apart from their high price these high alloy steels cannot be used for many purposes, for instance boiler tubes, on account of their Martensite structure in the rolling or forging state, and the difficulty of working them.

Separate technological tests, as for example the hard bending test for steam tubes (according to the resolutions of the German Steam Boiler Commission on regulations with regard to material and work for stationary boilers, of June 18, 1926), as also the rolling, etc. of the before-mentioned high alloy materials, meet with almost insuperable difficulties, apart from the difficult and almost impossible production of tubes.

40 High alloys of iron-aluminum, having content of more than 10% aluminum, and which are heat resisting up to more than 900° C., are also known, but these alloys are only used for castings, as 45 they cannot be rolled or forged.

In several prior patent specifications iron-aluminum alloys are described, all of which have high aluminum content (never under 5%) and high nickel and chromium contents. For example:

United States patent specification 1,633,805

|          | Per cent |
|----------|----------|
| Aluminum | 10 to 15 |
| Chromium | 5 55     |
| Nickel   | 30       |

United States patent specification 1,633,826

|          | Per cent   |
|----------|------------|
| Aluminum | 8 to 15 60 |
| Nickel   | 25         |
| Chromium | 7 to 15    |

British patent specification 220,006

Up to 40% chromium with high manganese, 65 nickel and tungsten contents. The addition of cobalt, copper and aluminum in small quantities is only incidentally mentioned as alloy constituents.

British patent specification 215,231

|          | Per cent   |
|----------|------------|
| Chromium | 15 to 35   |
| Aluminum | 5 to 12 75 |

As resistance to scaling up to 900° C. is always required it was necessary to use these high alloyed steels. There are however purposes for which it is desired to have resistance against scaling at lower temperatures. Ordinary iron begins to scale in an oxidizing atmosphere as low as 600° C. A soft low percentage alloy which would not show scaling at 700° to 800° C. would be an advance, as these temperatures are for many productions partly treatment and partly working temperatures.

The present invention is based on the results of exhaustive investigations carefully carried out over a long period in this direction, and which have led to a material which satisfies for example 90 the requirements of modern high capacity steam boilers. The intended increase of steam temperature to about 600° C. has hitherto been prevented for the want of suitable material, which not only had to be scale resisting but which could 95 be rolled without difficulty and which in every other respect would satisfy the various treatment and working requirements of the above mentioned technical tests. The material of the invention has properties which the high alloy, high tem- 100

perature resisting steels, apart from their high cost, did not possess.

The essence of the invention lies in the recognition that 2.7% of aluminum is sufficient as an alloy to make ordinary steel scale-resisting up to about 800° C., and that aluminum content as high as that made known by the before-mentioned proposed alloys, must be regarded for many purposes as disturbing or even as actually prejudicial. The economical progress shown in the price alone, will be easily recognized.

In contradistinction to the high alloy, high heat resisting steels, this low alloy aluminum-steel may be subjected without difficulty and without special precautionary measures to the most diverse punching and rolling processes (such as the Ehrhardt, Stiefel, Mannesmann etc.) and may for example be rolled into tubes.

Thus the invention relates to a steel alloy which is used in the rolled, drawn, punched or forged state and which is scale-proof up to 800° C., said steel comprising a low alloyed soft steel containing about 2.7 to 4%, or preferably 3 to 4% of aluminum. The balance of the alloy consists principally of iron in addition to the usual non-metallic constituents, which preferably are present in the relatively low amounts as hereinafter specified. Furthermore, it may contain, as will be seen more in detail from the following specification, such elements, which in respect to the solubility of the alpha-iron for the carbon, operate in a contrary manner to aluminum in a total amount up to about 2%. Each constituent of said type may be present in amounts lower than 1%. Silicon may be used in small amounts. Other alloying constituents are not intended to be present in the alloy in appreciable amounts which would influence the character of the alloy.

A further advance is the discovery that this steel, which is in itself coarse grained, may by suitable heat treatment be improved, that is, made tough and ductile. By heating, with subsequent quenching, from temperatures above 700° C. up to about 1000° C. and re-heating to 500° up to 750° C. a tough steel may be obtained. The technical tests on boiler tubes are more easily met and the steel may be drawn out for tubes of smaller diameters. It should be here mentioned, that unlike the usual heating, the first heating in the region of the solid solution should preferably last longer, in order to ensure the complete diffusion of the carbon in the interior of the aluminum-ferrite. As above a certain limit of concentration, which lies below about 2% aluminum, the gamma ( $\gamma$ ) phase is entirely suppressed and according to experiments made by the Kaiser-Wilhelm-Institute for the investigation of iron, only one holding point ( $A_e$  at 735° A at 732° C.) could be detected. It is not necessary in the improving process to quench the steel above 800° C.; as, with content above 2% aluminum, it is impossible to reach the field of the solid solution, but through the quenching a better distribution of the pearlite is obtained and besides even with longer subjection to heat, scaling is prevented. A further advantage of the steel produced by the new process is, that with it, such processes of treatment as hitherto necessitated special intermediate treatment for the purpose of removing scale (as for example treatment with acid), may now be carried out without such intermediate treatment.

Various methods of carrying out the new process are more fully described below:

75 1. For the production of scale-proof steels, but

which do not need to be specially tough, the following alloy is preferably chosen:

|            |                     |    |
|------------|---------------------|----|
| Carbon     | up to 0.4%          |    |
| Manganese  | about 0.20 to 0.80% | 80 |
| Phosphorus | below 0.02%         |    |
| Sulphur    | below 0.02%         |    |
| Silicon    | 0 to 0.8%           |    |
| Aluminum   | 2.7 to 4%           |    |

These low alloy aluminum steels may be rolled into plates, bars or shapes and made into tubes of large and small dimensions without difficulty, by the most diverse punching and rolling processes. They are scale-resisting up to 800° C., and are suitable, for instance, for gas generator retorts, for tubes in which a gaseous or fluid medium is to be heated, and for other purposes. With a tensile strength of about 40 to 50 kgs/mm<sup>2</sup> in the rolled state, the elongation was from 10 to 18%. They are easily electrically welded and are worked without difficulty.

2. A second way of carrying out the process is specially suitable for articles which should be tougher. A steel article produced according to the previously described process is subjected in the rolled state to an annealing or improving process, in which it is for example heated at 750° to 950° C., for a longer period than usual normalizing. The article is then quenched in water and tempered, but longer than usual, at about 500° to 750° C. If the heating is carried out as quickly as usual, only a partially fine structure is obtained, the carbon has not sufficient time to completely diffuse, as the aluminum in the alpha ( $\alpha$ ) iron operates against the diffusion of the carbon. A certain toughness may be obtained by simply heating at 600° to 700° C., which on account of the low cost, is preferable for objects not needing great ductility.

3. By means of another way of carrying out the process, a finer structure, and above all, more evenly distributed carbon contents, are at once obtained. For this, certain additions are required as alloy elements, which in respect of the solvent properties of the alpha ( $\alpha$ ) iron for the carbon, act in a contrary manner to aluminum. Exhaustive experiments have shown, that with quite small additions of chromium or manganese, or of both together, a finer grained structure may be obtained in the cast metal and consequently in the forged or annealed state also. Tungsten, molybdenum, vanadium, titanium etc. alone or jointly, act more strongly in this direction. These elements also act on the tensile properties in known manner. One or more elements should therefore be chosen, which, besides, producing a finer grain, also give the desired tensile strength. For instance the aluminum steel is alloyed with molybdenum or vanadium, or with both together, if a high range of heat resistance is required. Titanium is to be preferred for imparting shearing strength.

The forged state structure of this steel is considerably finer grained and more even, than without these additions. The alloy elements are given in each case.

4. In a further manner of carrying out the process, where it is desired to obtain great ductility, these steels are quenched down from about 800° C. and re-heated at 500° to 750° C., as mentioned earlier. A certain degree of toughness may be obtained by simply heating up these steels at 600° to 700° C., instead of quenching and tempering them.

The following tables show a few values, which

clearly indicate the improvement in the toughness depending on the alloy additions and the improving treatment. The high elastic limit as compared with the tensile strength is worthy of note, as it often reaches 80 per cent.

| Description and analysis | Treatment, degrees C.                |                                        |                                    |
|--------------------------|--------------------------------------|----------------------------------------|------------------------------------|
|                          | Elastic limits<br>kg/mm <sup>2</sup> | Tensile strength<br>kg/mm <sup>2</sup> | Elongation<br>% = 5d               |
| <i>Alloyed with</i>      |                                      |                                        |                                    |
| 3.26% aluminum           | 36.4<br>35.4                         | 46.5<br>44.2                           | 15.0<br>30.0                       |
| 2.7% aluminum            | 34.6                                 | 44.2                                   | 28.4                               |
| 0.8% chromium            | 33.0                                 | 48.2<br>44.7                           | 21.4<br>27.6                       |
| 2.8% aluminum            | 39.4                                 | 52.5                                   | 16.3                               |
| 0.8% chromium            | 35.8                                 | 51.8                                   | 28.8                               |
| 0.1% molybdenum          | 47.5                                 | 59.4                                   | 14.2                               |
| 0.1% tungsten            | 35.4                                 | 54.8                                   | 18.3                               |
| 3.6% aluminum            | 44.1                                 | 56.1                                   | 25.0                               |
| 0.7% chromium            | 39.7                                 | 54.0                                   | 24.2                               |
| 0.3% molybdenum          | 38.7<br>48.8                         | 52.2<br>59.9                           | 29.2<br>20.4                       |
|                          |                                      |                                        | Annealed at 940°.                  |
|                          |                                      |                                        | Quenched from 940°, tempered 650°. |
|                          |                                      |                                        | Quenched from 800°, tempered 650°. |
|                          |                                      |                                        | As delivered.                      |
|                          |                                      |                                        | Quenched from 940°, tempered 650°. |
|                          |                                      |                                        | As delivered.                      |
|                          |                                      |                                        | Quenched from 940°, tempered 650°. |
|                          |                                      |                                        | As delivered.                      |
|                          |                                      |                                        | Annealed 940°.                     |
|                          |                                      |                                        | Quenched from 940°, tempered 650°. |
|                          |                                      |                                        | Quenched from 800°, tempered 650°. |
|                          |                                      |                                        | Quenched from 940°, tempered 730°. |
|                          |                                      |                                        | Annealed at 680°.                  |

Below are further explanations with regard to the tables referring to the new process and the new material:

| No. | Appearance of fracture                     | Treatment degrees C.                         | Elongation % |
|-----|--------------------------------------------|----------------------------------------------|--------------|
| 1   | Rather coarse grained                      | Rolled                                       | 13.3         |
| 2   | Very coarse grained                        | Annealed at 940° air cooled                  | 15.0         |
| 3   | Fine grained, fibrous                      | Quenched from 940° tempered 1 hour at 730°   | 24.2         |
| 4   | Fine grained, fibrous, greater contraction | Quenched from 940° tempered 1/4 hour at 650° | 30.0         |
| 5   | Fibrous greatest contraction               | Quenched from 800° tempered 1 hour at 650°   | 28.4         |

The following remarks apply to other structures of such steels:

A fine grained micro-structure after quenching, similar to austenite, of a steel with 3% aluminum and 0.3% tungsten is extraordinarily

0

5

0

5

0

brittle in this condition. The carbon is completely in solution; the fracture is coarse crystalline. After tempering this quenched steel the carbon in the separate austenite fields separates out as cementite, the lamellæ of which are rather widely separated, so that a considerably higher carbon content, with more active etching, is shown. The elongation of the test bars (1=5d), which was 1.2% in the quenched state, has risen to 30.5%; and the contraction from 6.2 to 70.8%. 80 85

The object of the invention is further to produce material according to the various forms of carrying out the new process, suitable for making articles capable of resisting scale formation up to 800° C., especially tubes, the material consisting of low alloyed soft steel containing about 2.7% to 4% aluminum. In particular the invention comprises the use of this new material, utilizing its special properties, in particular as material for the making of such objects as may be produced by known rolling or drawing processes, as for the production of drawn or rolled tubes. Finally a part of the invention is the means to produce in particular superheater tubes, steam boiler and stay tubes, as well as other steam boiler components, especially for high pressure boilers, from a low alloy soft steel containing about 2.7 to 4% aluminum. 90 95 100

What I claim and desire to secure by Letters Patent of the United States is:

1. A rolled, drawn, punched or forged steel material, scale proof up to 800° C., which is made of a low alloyed soft steel containing about 2.8% of aluminum, about 0.8% of chromium, about 0.1% of molybdenum, and about 0.1% of tungsten, while the balance consists of iron besides the usual non-metallic constituents and is free from further alloying constituents. 110

2. A rolled, drawn, punched or forged steel material, scale proof up to 800° C., which is made of a low alloyed soft steel containing from about 2.7% to about 3.6% of aluminum, from about 0.7% to about 0.9% of chromium, from about 0.1% to about 0.5% of molybdenum, and from about 0.1% to 0.5% of tungsten, while the balance consists of iron besides the usual non-metallic constituents and is practically free from further alloying constituents. 115 120

HERMANN JOSEF SCHIFFLER.

135

135

130

135

140

145